# EUROPEAN PATENT APPLICATION

(11) **EP 1 796 124 A2**
(43) Date of publication of application: **13.06.2007**
(21) Application number: 06256244.2
(22) Date of filing: 07.12.2006
(51) Int. Cl.: H01J 17/49

(54) **Plasma display panels and methods for producing the same**

(30) Priority: 07.12.2005 KR 20050118647; 03.01.2006 KR 20060000585
(71) Applicant: LG Electronics Inc., Youngdungpo-Gu Seoul (KR)
(72) Inventor: Kim, Bo Hyun 531-1101 Sinan Apt., Suwon-si Gyeonggi-do, 443-811 (KR); Park, Min Soo 404 Hwasin Parkvill, Seoul, 137-070 (KR); Park, Deok Hai, Daegu, 700-441 (KR); Ryu, Byung Gil 2-102 SinHyundai Apt., Seoul (KR); Sim, Young Sung 105-903 Shinsung Apt., Gyeonggi-do, 449-772 (KR)
(74) Representative: Camp, Ronald

(57) **Abstract**

Disclosed is a plasma display panel with improved discharge characteristics. The plasma display panel comprises an upper panel and a lower panel integrally joined to the upper panel through barrier ribs wherein the upper panel includes a first protective film composed of a material having a work function lower than that of magnesium oxide and a second protective film formed on the first protective film and composed of magnesium oxide.

## Description

The present invention relates to plasma display panels. It more particularly relates to protective films of plasma display panels.

Plasma display panels comprise an upper panel, a lower panel, and barrier ribs formed between the upper and lower panels to define respective discharge cells. A major discharge gas, such as neon, helium or a gas mixture thereof, and an inert gas containing a small amount of xenon (Xe) are fill the discharge cells. When a high-frequency voltage is applied to produce a discharge in the discharge cells, vacuum ultraviolet radiation generated from the inert gas causes phosphors present between the barrier ribs to emit visible light, and as a result, images are created. Such plasma display panels have attracted more and more attention as next-generation display devices due to their small thickness and light weight.

FIG. 1 is a perspective view schematically showing the structure of a plasma display panel. As shown in FIG. 1, the plasma display panel comprises an upper panel 100 and a lower panel 110 integrally joined in parallel to and at a certain distance apart from the upper panel. The upper panel 100 includes an upper glass plate 101 as a display plane by which images are displayed and a plurality of sustain electrode pairs, each of which consists of a scan electrode 102 and a sustain electrode 103, arranged on the upper glass plate 101. The lower panel 110 includes a lower glass plate 111 and a plurality of address electrodes 113 arranged on the lower glass plate 111 so as to cross the plurality of sustain electrode pairs.

Stripe type (or well type, etc.) barrier ribs 112 for forming a plurality of discharge spaces, i.e. discharge cells, are arranged parallel to each other on the lower panel 110. A plurality of address electrodes 113, which act to perform an address discharge, are arranged in parallel with respect to the barrier ribs to generate vacuum ultraviolet radiation. Red (R), green (G) and blue (B) phosphors 114 are applied to upper sides of the lower panel 110 to emit visible light upon address discharge, and as a result, images are displayed. A lower dielectric layer 115 is formed between the address electrodes 113 and the phosphors 114 to protect the address electrodes 113.

An upper dielectric layer 104 is formed on the sustain electrode pairs 103, and a protective layer 105 is formed on the upper dielectric layer 104. The upper dielectric layer 104, which is included in the upper panel 100, becomes worn out due to the bombardment of positive (+) ions upon discharge of the plasma display panel. When this happens, short circuiting of the electrodes may be caused by metal elements, such as sodium (Na). Thus, a magnesium oxide (MgO) thin film acting as a protective layer 105 is formed by coating to protect the upper dielectric layer 104. Magnesium oxide sufficiently withstands the bombardment of positive (+) ions and has a high secondary electron emission coefficient, thus achieving a low firing voltage.

However, the protective layer of the conventional plasma display panel has the following problems.

Firstly, magnesium oxide can be used to form a highly sputtering-resistant protective film because it serves to improve the alignment, crystallinity and density of the protective film, and magnesium oxide exhibits better electrical properties. However, the power consumption of a plasma display panel comprising such a protective film still remains high.

Secondly, since magnesium oxide is highly hygroscopic, there is a possibility that phosphors may be discolored by discharge sputtering.

The present invention seeks to provide an improved plasma display panel.

Embodiments of the invention can provide plasma display panels comprising a protective film with a high secondary electron emission coefficient.

Embodiments of the invention can provide a protective film that can lower the firing voltage of plasma display panels comprising the protective film and that can reduce the power consumption of the plasma display panels.

Additional advantages and features of the invention will be set forth in part in the description which follows and in part will become apparent to those having ordinary skill in the art upon examination of the following or may be learned from practice of the invention.

In accordance with a first aspect of the invention, a plasma display panel comprises an upper panel and a lower panel integrally joined to the upper panel through barrier ribs wherein the upper panel includes a first protective film composed of a material having a work function lower than that of magnesium oxide and a second protective film formed on the first protective film and composed of magnesium oxide.

In accordance with another aspect of the invention, there is provided a method for producing a plasma display panel which comprises forming a dielectric layer on pairs of sustain electrodes included in an upper panel, forming a first protective film on the dielectric layer, and forming a second protective film on the first protective film wherein the first protective film is composed of a material having a work function lower than that of magnesium oxide and the second protective film is composed of magnesium oxide.

In accordance with another aspect of the invention, there is provided a plasma display panel comprising an upper panel and a lower panel facing each other through barrier ribs wherein the upper panel includes a first protective film composed of single-crystal magnesium oxide and a second protective film in the form of a thin film formed on the first protective film and composed of magnesium oxide.

In accordance with yet another aspect of the invention, there is provided a method for producing a plasma display panel which comprises forming a first protective film on a dielectric layer included in an upper panel and forming a second protective film in the form of a thin film formed on the first protective film wherein the first protective film is composed of single-crystal magnesium oxide and the second protective film is composed of magnesium oxide.

It is to be understood that both the foregoing general description and the following detailed description of the present invention are exemplary and explanatory and are intended to provide further explanation of the invention as claimed.

Embodiments of the invention will now be described by way of non-limiting example only, with reference to the drawings, in which:

FIG. 1 is a perspective view of a plasma display panel;

FIG. 2 is a schematic cross-sectional view of a plasma display panel according to a first embodiment of the invention; and

FIG. 3 is a cross-sectional view of a plasma display panel according to a second embodiment of the invention.

Wherever possible, the same reference numbers will be used throughout the drawings to refer to the same or like parts.

The embodiments of the invention to be described provide plasma display panels comprising a bilayered protective layer. Hereinafter, a layer formed on one surface of an upper dielectric layer will be referred to as a 'first protective film', and a layer formed on the first protective film will be referred to as a 'second protective film'.

A first embodiment of the invention will now be described with reference to FIG. 2.

Only the upper panel of a plasma display panel is shown in FIG. 2. As shown in FIG. 2, an upper dielectric layer 275 is formed in the upper panel on a substrate 270, and a first protective film 280a and a second protective film 280b are sequentially formed on the upper dielectric layer 275. The first protective film 280a is formed on the upper dielectric layer 275 and is composed of a material having a work function lower than that of magnesium oxide. The second protective film 280b is formed on the first protective film 280a and is composed of magnesium oxide. It is preferred, but not essential to the invention in its broadest aspect, that the first protective film 280a be composed of a material having a work function not higher than 3 eV and having an energy band gap smaller than that of magnesium oxide. That is, since the first protective film 280a is composed of a low-work function material, it can emit an increased number of secondary electrons. Further, in the present embodiment the material constituting the first protective film 280a has a density equal to and greater than CaO. Specifically, in the present non-limiting embodiment, the material constituting the first protective film 280a has a density of 3.37 g/cm³. In this embodiment, the material constituting the first protective film has a higher density than magnesium oxide. However this is not essential to the invention in its broadest aspect. Examples of materials that have a lower work function than magnesium oxide include BeO, CaO, SrO and BaO. The work function, density and energy band gap values of these materials are listed in Table 1.

**TABLE 1**

| Material | Density (g/cm³) | Work function (eV) | Energy band gap (eV) |
|---|---|---|---|
| MgO | 3.65 | 3.1-4.4 | 7.30 |
| CaO | 3.37 | 1.76 | 5.60 |
| SrO | 4.70 | 1.27 | 5.70 |
| BaO | 4.96 | 0.99 | 1.85-2.08 |

Common protective films commonly have a thickness of 500 to 800 nm. In the first embodiment, the first protective film 280a has a thickness of 200 to 800 nm and the second protective film 280b has a thickness of 5 to 300 nm. That is, the second protective film 280b composed of the same material as conventional protective films is formed to a small thickness on a surface in contact with discharge spaces to prevent the upper dielectric layer 275 from becoming worn out due to bombardment by positive (+) ions.

The second protective film 280b composed of magnesium oxide is formed with a small thickness so that electrons emitted from the first protective film 280a can be satisfactorily supplied to discharge spaces. The first protective film 280a may, as in the present embodiment, be formed from particles or aggregates of the particles. In this case, the first protective film 280a can be formed on portions of the surface of the upper dielectric layer 275. Since the second protective film 280b in the form of thin film is formed on the first protective film 280a, the protective film 280b conforms with the surface topology of the first protective film 280a. This conformity of the protective films leads to an increase in the area of the magnesium oxide applied to the first protective layer 280a so that an increased number of secondary electrons can be emitted upon discharge of the plasma display panel. In the present exemplary embodiment the magnesium oxide constituting the second protective film 280b has a thickness of 10 to 100 nm. However this is not essential to the invention in its broadest aspect.

The first protective film needs to have a low secondary electron emission coefficient in order to reduce the firing voltage of the panel. The secondary electron emission coefficient of a material is intimately associated with the work function and the energy band gap of the material. Specifically, the smaller the energy band gap of a material, the lower the secondary electron emission coefficient of the material. Alkaline earth metals other than magnesium oxide have a lower work function than magnesium oxide and a smaller energy band gap than magnesium oxide, and have a density similar to or greater than magnesium oxide. Gd₂O₃ and Sc₂O₃, which are rare earth oxides, have a much higher density and a smaller energy band gap than magnesium oxide. Accordingly, in the present exemplary embodiment an alkaline earth metal selected from CaO, SrO, BaO and BeO or a rare earth oxide selected from Gd₂O₃ and Sc₂O₃ is used to constitute the first protective film 280a. However this is not essential to the invention in its broadest aspect.

A dopant may be added to the first protective film 280a or the second protective film 280b to lower the porosity and increase the density of the protective film 280a or 280b. However this is not essential to the invention in its broadest aspect. As a result, attachment of impurities to the surface of the magnesium oxide thin film can be prevented and the firing voltage of the plasma display panel can be lowered. Silicon or lead may be used as the dopant. Other examples of the dopant include aluminum (Al), boron (B), barium (Ba), indium (In), zinc (Zn), phosphorus (P), gallium (Ga), germanium (Ge), scandium (Sc), and yttrium (Y). The dopant may be formed on the first protective film and/or the second protective film. It is preferable, but not essential to the invention in its broadest aspect, that an oxide powder of the dopant be added to the protective film and homogeneously mixed with the magnesium oxide within the protective film. Examples of suitable oxides include Al₂O₃, B₂O₃, SiO₂, P₂O₅, Ga₂O₃, GeO₂, Sc₂O₃, and Y₂O₃.

A method for forming the first protective film will be described below.

The first protective film 280a is formed by a process selected from sputtering, ion plating and e-beam deposition. Sputtering is widely employed at present to form various thin films. According to a sputtering process, particles having a high energy (> 30 eV) collide with a target to transfer the energy to the target atoms, after which the target atoms are emitted from the target to form the first protective film 280a. Ion plating is a general name for a combination of vacuum evaporation and sputtering. In ion plating, glow discharge is produced when a high voltage is applied under a high vacuum to form a plasma and parts of vaporized atoms are ionized. These phenomena are utilized to form the first protective film 280a. According to e-beam deposition, the first protective film 280a is formed by heating a crystal, e.g., a BeO crystal, to a high temperature to physical energy, i.e. by using physical energy. While E-beam deposition is the most preferred process in view of uniformity of the film. Other processes may be employed to form the first protective film. Examples of such processes include liquid-phase deposition and vapor phase oxidation.

An explanation of a method for producing the plasma display panel according to the first embodiment will now be given.

First, pairs of sustain electrodes are formed on a substrate. A dielectric layer is formed on the substrate and the pairs of sustain electrodes, and then a first protective film and a second protective film are sequentially formed on the dielectric layer. The first and second protective films are the same as the protective films of the plasma display panel according to the first embodiment. That is, the first and second protective films can be formed by any convenient process such as sputtering, ion plating, e-beam deposition or liquid-phase deposition.

An explanation of the second embodiment will be given with reference to FIG. 3.

Only an upper panel of the plasma display panel is shown in FIG. 3. As shown in FIG. 3, pairs of sustain electrodes 390, an upper dielectric layer 375 and a protective layer are sequentially formed on an upper substrate 370. The protective layer has a bilayer structure consisting of a first protective film 380a and a second protective film 380b. The first protective film 380a is composed of single-crystal or polycrystalline magnesium oxide and preferably single-crystal magnesium oxide. In the present exemplary embodiment the first protective film 380a may be formed using single-crystal magnesium oxide particles or aggregates of the particles. That is, the magnesium crystal particles are formed in an island shape, and as a result, the first protective film 380a has an irregular shape due to the difference in height between portions where the magnesium crystal particles or aggregates of the particles are formed and portions where the magnesium crystal particles or aggregates of the particles are not formed. The second protective film 380b is formed to a uniform thickness on the first protective film 380a, and thus it also has an irregular shape due to the irregular shape of the first protective film 380a.

In the present non-limiting embodiment the single-crystal magnesium oxide constituting the first protective film 380a has a size of 10 to 100 nm. In this embodiment the first protective film 380a has a thickness of 500 to 800 nm, and the second protective film 380b has a thickness of 5 to 300 nm. If the shape of the magnesium oxide crystal is a sphere, the size of the magnesium oxide crystal refers to the diameter of the sphere. If the shape of the magnesium oxide crystal is a cube, the size of the magnesium oxide crystal refers to the length of one side of the cube. The single-crystal magnesium oxide constituting the first protective film 380a serves to protect the upper dielectric layer 375, and at the same time, to emit secondary electrons. However, instead of crystalline magnesium oxide, a material having a secondary electron emission coefficient higher than that of magnesium oxide may be used to constitute the first protective film 380a.

The material having a secondary electron emission coefficient, which arises from bombardment by positive (+) ions, higher than that of magnesium oxide, may be single-crystalline or polycrystalline. Examples of such single-crystal materials include KBr, KCl, KI, NaBr, NaCl, NaF, NaI and LiF, and examples of such polycrystalline materials include CsCl, KCl, KI, NaBr, NaCl, NaF, NaI, LiF, RbCl, Al₂CO₃, BaO, BeO, BaF₂, CaF, BiCs₃, GeCs, Rb₃Sb, and SbCs₃. The secondary electron emission coefficient of magnesium oxide varies depending on the measurement conditions. Magnesium oxide is measured to have a secondary electron emission coefficient lower than 1 under routine conditions. The secondary electron emission coefficients of the single-crystal materials are as follows: KBr = 14, KCl = 12, KI = 10, NaBr = 24, NaCl = 14, NaF = 14, NaI = 19, and LiF = 8.5. The secondary electron emission coefficients of the polycrystalline materials are as follows: CsCl = 6.5, KCl = 7.5, KI = 5.6, NaBr = 6.3, NaCl = 6.8, NaF = 5.7, NaI = 5.5, LiF = 5.6, RbCl = 5.8, Al₂CO₃ = 2-9, BaO = 2.3-4.8, BeO = 3.4, BaF₂ = 4.5, CaF₂ = 3.2, BiCs₃ = 6, GeCs = 7, Rb₃Sb = 7.1, and SbCs₃ = 6. The secondary electron emission coefficient of a material is defined as the number of electrons ejected from the material when one electron collides with the material.

As explained earlier, when the protective films are non-planar, the area of the magnesium oxide applied to the first protective layer 380a is increased so that an increased number of secondary electrons can be emitted upon discharge of the plasma display panel. Alternatively, when the surfaces of the protective films are irregular, the electric field becomes concentrated on portions protruding from the protective films toward discharge spaces to promote the emission of secondary electrons, resulting in a reduction in the firing voltage of the plasma display panel.

An explanation of a method for producing the plasma display panel according to the second embodiment will be provided below.

First, pairs of sustain electrodes and a dielectric layer are sequentially formed on a glass substrate included in an upper panel. Then, single-crystal or polycrystalline magnesium oxide particles or aggregates of the particles are formed on the dielectric layer to form a first protective film. The single-crystal magnesium oxide constituting the first protective film has a size of 10 to 100 nm. The first protective film has a thickness of 500 to 800 nm. The first protective film is preferably formed by a process selected from screen printing, green sheet lamination, inkjet printing and liquid-phase deposition. However this is not essential to the invention in its broadest aspect and any other suitable process known to the skilled person may be employed.

Subsequently, a second protective film in the form of a thin film is formed on the first protective film. In the present embodiment the second protective film has a thickness of 5 to 300 nm. The second protective film in the form of a thin film is in the present embodiment formed to a uniform thickness. Any process, such as e-beam deposition, sputtering, ion plating, green sheet lamination or coating, suitable for the formation of a thin film, may be employed to form the second protective film.

The bilayer structure of the protective films of the plasma display panel and the increased area of the magnesium oxide applied to the first protective film 380a enable the emission of an increased number of secondary electrons upon discharge of the plasma display panel.

It will be apparent to those skilled in the art that various modifications and variations can be made to the described embodiments without departing from the scope of the invention. Thus, it is intended that the present invention covers the modifications and variations of this invention provided they come within the scope of the appended claims. For example while ranges of values of dimensions of layers and particle sizes have been given for the purposes of illustration, the skilled person will appreciate that other dimensions may be used according to the requirements of a particular application of the invention. Likewise materials other than those explicitly referred to and having suitable properties may be used.

## Claims

1. A plasma display panel comprising an upper panel and a lower panel integrally joined to the upper panel through barrier ribs wherein the upper panel includes a first protective film composed of a material having a work function lower than that of magnesium oxide and a second protective film formed on the first protective film and composed of magnesium oxide.

2. The plasma display panel according to claim 1, wherein the material having a work function lower than that of magnesium oxide is selected from CaO, SrO, BaO and BeO.

3. The plasma display panel according to claim 1 or 2, wherein the first protective film is formed from particles or aggregates of the particles.

4. The plasma display panel according to any preceding claim, wherein the first protective film is formed on portions of the surface of an upper dielectric layer included in the upper panel.

5. The plasma display panel according to any preceding claim, wherein the second protective film is in the form of a thin film.

6. The plasma display panel according to any preceding claim, wherein the magnesium oxide constituting the second protective film has a thickness in the range of 10 to 100 nm.

7. The plasma display panel according to any preceding claim, wherein the first protective film is composed of a material having a work function not higher than 3 eV.

8. The plasma display panel according to any preceding claim, wherein the first protective film is composed of a material having an energy band gap smaller than that of magnesium oxide.

9. The plasma display panel according to any preceding claim, wherein the first protective film is composed of a material having a density not lower than that of CaO.

10. The plasma display panel according to any preceding claim, wherein at least one protective film selected from the first protective film and the second protective film contains at least one dopant.

11. The plasma display panel according to claim 10 in which the dopant comprises silicon (Si) and/or lead (Pb).

12. A method for producing a plasma display panel, the method comprising forming a dielectric layer over pairs of sustain electrodes included in an upper panel, forming a first protective film on the dielectric layer, and forming a second protective film on the first protective film wherein the first protective film is composed of a material having a work function lower than that of magnesium oxide and the second protective film is composed of magnesium oxide.

13. The method according to claim 12, wherein the first protective film is formed by a process selected from sputtering, ion plating and e-beam deposition.

14. A plasma display panel comprising an upper panel and a lower panel facing each other through barrier ribs wherein the upper panel includes a first protective film composed of single-crystal magnesium oxide and a second protective film in the form of a thin film formed on the first protective film and composed of magnesium oxide.

15. The plasma display panel according to claim 14, wherein the first protective film is formed using aggregates of single-crystal magnesium oxide particles so as to have an irregular surface.

16. The plasma display panel according to claim 14 or 15, wherein the second protective film is formed to a uniform thickness to have an irregular surface.

17. The plasma display panel according to any one of claims 14 to 16, wherein the first protective film is composed of a single-crystal material selected from KBr, KCl, KI, NaBr, NaCl, NaF, NaI, and LiF.

18. The plasma display panel according to any one of claims 14 to 16, wherein the first protective film is composed of a polycrystalline material selected from CsCl, KCl, KI, NaBr, NaCl, NaF, NaI, LiF, RbCl, Al₂CO₃, BaO, BeO, BaF₂, CaF, BiCs₃, GeCs, Rb₃Sb, and SbCs₃.

19. A method for producing a plasma display panel, the method comprising forming a first protective film on a dielectric layer included in an upper panel and forming a second protective film in the form of a thin film formed on the first protective film wherein the first protective film is composed of single-crystal magnesium oxide and the second protective film is composed of magnesium oxide.

20. The method according to claim 19, wherein the first protective film is formed by a process selected from screen printing, green sheet lamination, inkjet printing, and liquid-phase deposition.

21. The method according to claim 19 or 20, wherein the second protective film is formed by a process selected from e-beam deposition, sputtering, ion plating, green sheet lamination, and coating.
